

## UNITED STATES PATENT OFFICE

2,104,427

## METHOD OF PRETREATING IRON SURFACES

Alexander Kreidl, Vienna, Austria

No Drawing. Application December 7, 1933, Serial No. 701,341. In Austria December 7, 1932

6 Claims. (Cl. 91—70)

The present invention relates to a method of enameling the surface of metals, such as iron, steel, cast iron etc.

The invention is based on the recognition of two factors independent of each other, viz: For one thing, it has been found from an extraordinarily large number of systematically conducted experiments that to achieve a particularly intimate adhesion of enamel to iron, steel, cast iron, etc., the formation of an intermediate film of spinel-like composition on the iron surface to be enamelled is essential; this film may practically be as thin as desired. In general, and without detailed reference to the structures which have been recently found by X-ray experiments, spinels are compounds which form between monoxides and sesquioxides in a state of incandescence. These two spinel components are, of course, capable of being yielded by iron itself, but it is just this property which, it has been found, make special precautions necessary. I have ascertained, surprisingly, that satisfactory adherence can only be obtained if the iron surface to be enamelled, does not contribute from the sesquioxide state to the formation of the film; the iron surface should be protected to the greatest possible extent from oxidizing to ferric oxide. Obviously, such oxidation would effect a loosening of the iron base, a process which cannot be remedied or cured, and which brings in its train (even against the action of the subsequently applied enamel) stripping, rupturing, flaking and other similar undesirable results.

The technical utilization of these two novel factors constitutes the essence of the present invention, which comprises a method for the enamelling (without using any ground enamel) of iron, steel, cast iron or the like in which the surface to be enamelled is pretreated in such a manner that a film of the character above defined may form on such surface; while at the same time the simultaneous formation of ferric oxide on the iron base is inhibited to the maximum degree.

I find that I accomplish the object of my invention by heating the iron surface to be enamelled in the presence of a coating containing a metal-oxide-metal-sesquioxide mixture or combination, with the addition of flux, in an atmosphere poor in oxygen in comparison with air. Under these conditions the film formation takes place with simultaneous attainment of the desired surface protection. If it be desired to enhance such surface protection, which might be desirable under certain circumstances, suitable

measures to that end may be taken as follows:—the heating period is limited to just that short duration which is necessary for the formation of the spinel film, and it has been found in practice that a heating period of but very few minutes suffices. The heating temperature is desirably adjusted to between about 750° C. and about 800° C.

As to the heating atmosphere itself, it developed in the course of practical operation, by way of the admixture of generator gas or the like, that the reduction of the oxygen content to approximately one-third of the normal content is advantageous. If the metals to be enamelled contain adequate quantities of reducing substances, i. e. oxygen-consuming substances, such as carbon, hydrogen, hydrocarbons and the like, then under proper conditions the requisite lowered content of oxygen may be automatically adjusted so that the heating process is then limited to heating under exclusion of air.

The metal surfaces to be enamelled, before their introduction into the furnace, are moistened with the metal compounds by the heating of which the spinel like conversion is to be effected, the moistening being effected either by immersing the surface in a liquid containing these metal compounds, by spraying etc. In order that the spinel film may smoothly and gaplessly adhere to the metal surface, the moistening fluid has preferably added to it a suitable flux, such as boric acid or fluorspar. It will be obvious that appropriate moistening or wetting substances are not only such which act directly as spinel components, but also such compounds out of which the spinel components are capable of forming at the temperature of incandescence. The purpose of my invention would not be served, and indeed would be defeated, if the metal surface to be enamelled were pretreated with the metal compounds of the present invention without incandescence or by heating in an ordinary atmosphere.

As the rust which usually adheres to iron surfaces is an excellent spinel former, it may be made useful and advantageous in the present process by assigning to the rust the role or function of one of the spinel components in the heating action. This will be recognized as an extraordinarily advantageous feature of the present invention because, thanks to the circumstance that rusty surfaces of any kind may be subjected to the process not only without detriment but with positive advantage, the present process is the first in the art which permits

the enamelling operation to be carried out without previous rust removal, thus dispensing with the pickling process and all its attendant evils in this art. The importance and value of this phase of the invention, in its simplification, improvement and cheapening of enamelling procedure cannot be overestimated.

The method of my invention may be carried out in practice in a considerable variety of ways. 10 For example, unpickled iron ware with or without rust adhering thereto, is wetted with a fluid containing to 100 parts of water, five parts of  $Fe_2O_3$ , four parts of  $NiO$ , twenty parts of  $CaF_2$ , forty five parts of boric acid and ten parts of 15 clay, or is wetted with a fluid containing to 100 parts of water ten parts of  $Fe_2O_3$ , six parts of  $MnO$ , twenty parts of  $CaF_2$ , thirty parts of boric acid and seven parts of clay; and after gentle 20 drying the article is heated seven minutes in a furnace at a temperature of from 785° to 795° C., the atmosphere prevailing in the furnace having its oxygen content reduced to one-fourth or one-fifth the normal content by the admixture therewith of generator or other exhaust gases, 25 whereupon the surface having the extremely thin film thereon is enamelled in a single operation.

I claim:

1. Method of pre-treating iron, steel, cast-iron and the like, for enamelling purposes, which 30 method comprises the steps of applying to the metal surface to be pretreated a combination

of flux with iron sesquioxide, and a monoxide selected from the group consisting of iron monoxide, nickel monoxide and manganese monoxide, heating said surface in an atmosphere containing such an amount of oxygen that substantially no oxidation of the metal of the said surface proper to iron sesquioxide occurs and cooling the surface, whereby a rough coating is produced which adapts said metal surface for enamelling. 5

2. The method claimed in claim 1, in which 10 said combination comprises substantially the following proportion of substances: 5 parts of  $Fe_2O_3$ , 4 parts of  $NiO$ , 20 parts of  $CaF_2$ , 45 parts of boric acid and 10 parts of clay for 100 parts of water.

3. The method claimed in claim 1, in which 15 said combination comprises substantially the following proportion of substances: 10 parts of  $Fe_2O_3$ , six parts of  $MnO$ , 20 parts  $CaF_2$ , 30 parts boric acid and 7 parts of clay to 100 parts of 20 water.

4. The method claimed in claim 1, in which the oxygen content of the atmosphere present during the heating step amounts to one-third 25 of that present in ordinary atmosphere.

5. The method claimed in claim 1, in which the heating step is performed at temperatures ranging between 750° and 800° C.

6. The method claimed in claim 1, in which the iron surface to be pre-treated contains rust. 30

ALEXANDER KREIDL.